

Feb. 27, 1951

C. S. FRANCIS, JR

2,543,101

COMPOSITE FIBROUS PRODUCTS AND METHOD OF MAKING THEM

Filed July 20, 1944

2 Sheets-Sheet 1



INVENTOR.  
Carleton S. Francis  
BY  
Carl A. Castellan  
ATTORNEY

Feb. 27, 1951

C. S. FRANCIS, JR

2,543,101

COMPOSITE FIBROUS PRODUCTS AND METHOD OF MAKING THEM

Filed July 20, 1944

2 Sheets-Sheet 2



INVENTOR.  
Carleton S. Francis  
BY  
Carl A. Castellan  
ATTORNEY

## UNITED STATES PATENT OFFICE

2,543,101

COMPOSITE FIBROUS PRODUCTS AND  
METHOD OF MAKING THEMCarleton S. Francis, Jr., West Harwich, Mass.,  
assignor to American Viscose Corporation, Wil-  
mington, Del., a corporation of Delaware

Application July 20, 1944, Serial No. 545,865

19 Claims. (Cl. 154—101)

1

This invention relates to composite products comprising at least one layer of prefabricated textile material and at least one layer of felt-like material, and in which one surface of at least one felt-like layer is exposed and the other surface is securely and substantially permanently anchored to a textile layer.

The present application is a continuation-in-part of my pending applications Serial No. 300,-876, filed October 23, 1939, now Patent No. 2,-459,803, Serial No. 405,102, filed August 1, 1941, now Patent No. 2,483,404, and Serial No. 530,553, filed April 11, 1944, now Patent No. 2,437,689.

In said prior applications there are disclosed various fibrous products, such as textiles, felts, and papers formed from a mixture of at least two types of products, one of which is potentially adhesive, and a process of forming fibrous products from such mixtures of fibers by rendering the potentially adhesive fibers in the mixture tacky to bind fibers in the product. According to the teachings of those applications there may be obtained felt-like fibrous bats or similar masses which are thick and soft and characterized by extremely low density and high porosity, or stiffer and firmer, more boardlike products may be obtained which are relatively non-porous or substantially impermeable, depending upon the percentage of potentially adhesive fibers present and/or the degree of activation thereof, that is, whether merely softened to the extent that they engage and interlock with each other and with the non-adhesive fibers, or are softened to the point where they lose their fibrous structure and flow to form a continuous film of binding material. Those prior applications further disclose methods of reinforcing the fibrous felt-like bats by anchoring the same to a textile material.

It is the general object of the present invention to provide felt-like fibrous bats of the type disclosed in my copending applications aforementioned of advantageous properties and a wide scope of usefulness. Another object is to provide such felt-like products with additional support or reinforcement. Still another object is to provide such products which combine in a single structure the properties of thickness, low density and high permeability, with the strength and toughness normally associated with products of greater density and a lower degree of permeability. Another object is to provide felt-like products comprising bats or the like which are capable of withstanding severe flexing or bending stresses and strains without damage to the interfelted structure of the bat. Still another object is to pro-

2

vide composite products of the type aforesaid, in which at least some of the fibers comprising the felt-like bat are extremely short and less than normal feltable length, i. e. fibers which cannot be felted by conventional procedures. A still further object is to provide composite products of the type mentioned, in which the non-adhesive fibers comprising the felt-like bat comprise wool stock, and which products have the properties of a high quality first-grade wool felt, such as hand, heat-insulating properties, volume or bulk, strength, etc. Still a further object is the provision of artificial leather articles closely simulating real leather products.

15 These and other objects are achieved by the present invention in accordance with which a composite product is formed from at least one felt-like bat or web, comprising potentially adhesive fibers and non-adhesive fibers, and a supporting or reinforcing textile fabric to which the body of the bat or web is bonded or anchored, so as to leave at least one exposed surface exhibiting felt-like characteristics, the fibers in the bat or web being bonded together due to activation of 20 the potentially adhesive fibers to a tacky condition.

25 The term "textile fabric" includes textiles made by any mode of associating yarns, such as weaving, knitting, netting, lacing, crocheting, or braiding. Such fabrics will be hereinafter referred to generally as textile fabrics comprising interlaced yarns. The fabric may comprise potentially adhesive fibers, non-adhesive fibers, or mixtures of the two types.

30 35 By potentially adhesive is meant those fibers which are capable of being rendered adhesive upon the application of heat either alone or in conjunction with swelling or solvent agents. By "non-adhesive" is meant those fibers which are not rendered adhesive by the treatment used in activating the potentially adhesive fibers.

40 45 The fibers present in the felt-like layer, and which may also comprise the textile fabric reinforcement may be composed of a wide variety of materials, and may comprise any material capable of being formed into fibers which have an inherent tackiness upon heating to temperatures below that at which the non-adhesive fibers are damaged or rendered tacky and which are non-tacky at room temperature. Examples of the potentially adhesive fibers include thermoplastic fibers, such as those of cellulose acetate or other cellulose esters and ethers or mixed esters, such as cellulose acetate propionate or cellulose acetate butyrate, in plasticized condi-

tion; also, resins, either permanently thermoplastic or thermosetting but in the thermoplastic state, formed by the polymerization or condensation of various organic compounds such as coumarone, indene or related hydrocarbons, vinyl compounds, styrene, sterols, phenol-aldehyde resins either unmodified or modified with oils, urea-aldehyde resins, sulfonamide-aldehyde resins, polyhydric alcohol-polybasic acid resins, drying oil-modified alkyd resins, resins formed from acrylic acid, its homologues and their derivatives, sulfurolefine resins, resins formed from dicarboxylic acids and diamines (nylon type); synthetic rubbers and rubber substitutes, herein called "resins" such for example as polymerized butadiene, olefine polysulfides, isobutylene polymers, chloroprene polymers; and fibers formed from a resin comprising the product of copolymerizing two or more resins, such, as copolymers of vinyl halide and vinyl acetate, copolymers of vinyl halide and an acrylic acid derivative; and also a mixture of resins, such as a mixture of vinyl resins and acrylic acid resins or methacrylic acid resins, a mixture of polyolefine resins and phenol-aldehyde resins, or a mixture of two or more resins from the different classes just named. There may be employed also fibres made from rubber latex, crepe rubber, gutta percha, balata, and the like.

Further, the fibers may be mixtures of the cellulose derivatives with resins or rubber, such for example, as a mixture of cellulose nitrate and an acrylic acid resin, or a mixture of benzyl cellulose and a vinyl resin, or a mixture of ethyl cellulose and shellac.

A preferred class of vinyl resins from which the fibers may be formed are the copolymers of vinyl chloride with vinyl acetate or vinyl cyanide and after-chlorinated copolymers of vinyl chloride and vinyl acetate.

The resins above mentioned may be classified as:

(a) Heat non-convertible resins such for example as glycol polybasic acid resins, vinyl resins (particularly those of the preferred class above) and the acid type phenolaldehyde resins, and the like.

(b) Heat-convertible or thermosetting resins such for example as glycerol-polybasic acid resins, polyolefine resins, phenol aldehyde resins and the like.

(c) An element-convertible resin (which becomes infusible through the action of certain elements, such as oxygen and sulfur) such for example as glycerol-polybasic acid-drying oils resins and olefine-sulfur resins.

Among the non-adhesive fibers which may be used are wood pulp fibers, cotton, flax, jute, kapok, silk, "wool stock," "leather dust" and the like, or synthetic fibers of cellulosic compositions, such as a cellulose or regenerated cellulose, cellulose derivatives, such as cellulose esters, mixed cellulose esters, cellulose ethers, mixed cellulose ethers, cellulose hydroxy-ethers, cellulose carboxy-ethers, cellulose ether-xanthates, cellulose xanthophatty acids, cellulose thiourethanes; natural and synthetic rubber and derivatives thereof; alginic acid, gelatine, casein; mineral fibers such as spun glass, asbestos, mineral wool and the like; fibers made of natural and synthetic resins which should be of such type that they are not rendered tacky when the activatable fibers are rendered tacky by heating; and the fibers made by slitting, cutting, or shredding non-fibrous films, such as waste cellophane.

The fiber-forming material from which the fibers are produced may contain added agents for obtaining special effects. For example, the parent fiber-forming material for the potentially adhesive fibers may contain hardening agents in the case of resins, for instance; while the fiber-forming material for either the potentially adhesive or the non-adhesive fibers may contain latent activating agents, dyes, pigments, mothproofing agents, fire-proofing agents, water-proofing agents, and the like.

The fibers may be pre-formed in any suitable manner. Thus, either type of fiber may be obtained by cutting previously formed continuous filaments to the desired length, or, in the case of the potentially adhesive fibers or of the non-adhesive fibers when prepared from organic film-forming material, the fibers may be pre-formed by dispersing, such as by spraying, the fiber-forming material while in flowable condition, that is, in solution, plastic, or molten condition, under sufficient pressure to form a multiplicity of fibers, into a setting fluid, e. g. a liquid or a gaseous atmosphere, as taught in my copending application Serial No. 381,292, filed March 1, 1941, now Patent No. 2,357,392.

The fibers may be of any length, and the non-adhesive fibrous material may comprise those fibers or fibrils which occur in waste products, such as cotton linters, shear flock, that is the fuzz removed from fabrics and felts during shearing operations, so-called "leather dust" or "leather-flock" that is, short leather fibers obtained by shaving down leather, the short fluffy waste thrown out of carding and/or combing machines, wool stock or waste, the waste from reeling, warping, winding, weaving, and cap bottoms, the waste from slubbing, roving, and wool tops, and in fact, all short fibers or fibrils which ordinarily do not find use in the manufacture of commercial products.

The felt-like bat may be formed by commingling the two types of fibers in any appropriate manner, as by carding, blowing in accordance with the teachings of my co-pending application Serial No. 530,953, filed April 14, 1944, now abandoned, or the potentially adhesive fibers may be formed by spraying a suitable fiber-forming composition into a chamber containing a setting fluid, the non-adhesive fibers being separately blown into or formed in the same chamber, so that they are associated with the potentially adhesive fibers concurrently with formation of the latter, as taught in my above mentioned application Serial No. 381,292, filed March 1, 1941, now Patent No. 2,357,392.

The commingled fibers are deposited or collected in the form of a bat or web in which the fibers may extend in haphazard relation without any substantial amount of parallelism, or the fibers in the bat may have some degree of accidental or intentional parallelism, such as that resulting from carding, for example.

Composite products in which the felt-like mass or bat is anchored to one or both sides of a textile fabric support may be produced in a variety of ways, such as by napping, needling, or plating the felt-like bat on the fabric.

For example, the product may be a "woven" felt, in which the basis is a woven construction of voluminous yarns comprising potentially adhesive and non-adhesive fibers and which has a full nap or pile which is felted until the woven structure is obscured. After the woven construction is shrunk and the nap felted in the usual manner,

the felt is subjected to heat to render the resin fibers tacky which effects an adhesion or bonding of the felted nap fibers.

The bat may also be pre-formed and "needled" or "plated" to the textile fabric reinforcement. In this case, the potentially adhesive fibers and the non-adhesive fibers may be commingled and the mixture is permitted to deposit, or is caused to be collected in the form of a bat or web. Such pre-formed bats or webs may be applied and then anchored to the fabric in a subsequent step in the procedure of manufacturing the new final reinforced felt structures. If the bat is pre-formed, it may be desirable to partially activate the potentially adhesive fibers to effect a preliminary binding together of the mixed fibers and permit handling of the web without damage thereto.

Alternatively, the potentially adhesive fibers and non-adhesive fibers comprising the felt-like bat may be commingled, if desired, simultaneously with formation of the potentially adhesive fibers, and the fibers may be deposited concurrently with commingling thereof, on the surface of the textile fabric to which anchoring is intended, and this latter procedure constitutes the preferred embodiment of the invention.

The anchoring may be the result solely of bonding between the potentially adhesive fibers in the bat or web (and/or fabric) obtained by appropriate activation, or it may be the result of the use of a separate layer of adhesive for this purpose interposed between the fabric and the bat or web. Alternatively, a thin continuous film, or a web of fibers, of a thermoplastic material which may be of the same or different composition as the potentially adhesive fibers in the bat or web may be used as the adhesive layer and may be rendered adhesive for bonding the components of the product at the same time as the fibers in the web or bat and/or fabric are activated. When such a thin continuous film or web of fibers is used, it may be disposed between the fabric and bat or it may be placed on the side of the fabric opposite the bat, activation in such case causing the penetration of such film or fibers through the interstices of the fabric or conversely the projection of the bat or main web through the fabric interstices to join the components into a unitary product. The use of a film applied by coating, spraying, or impregnating, may serve to seal the fabric surface of the product or provide a sealing membrane within the body of the product when disposed centrally therein.

Among the methods which may be used for the activation of the fibers (and the adhesive layer when it is of a potentially adhesive material) are the following, which methods may be practiced singly or in combination.

(a) When the potentially adhesive fibers are thermoplastic they may be activated by heat applied with or without pressure, and a preferred method of activation is to blow dry hot air through the product. In treating webs of considerable thickness the air may be blown first in one direction and then in the opposite direction through the web to avoid non-uniform activation and to minimize dislocation of the fibers in the web.

(b) The potentially adhesive fibers may be activated by applying to the fibrous mixture a solvent or swelling agent or mixtures thereof with diluents, under such conditions of concentration and temperature as to render the potentially adhesive fibers tacky. For example, fibers of or-

ganic cellulose derivatives such as cellulose esters may be rendered adhesive by solvents such as acetone, ethyl acetate, butyl acetate, and the like.

(c) A latent activating agent may be combined with the potentially adhesive fibers and/or with the non-adhesive fibers and the agent may be rendered active by a subsequent treatment, such as by treatment with chemical agents, heat or irradiation, thus producing a simultaneous activation of the potentially adhesive fibers in selected areas. For example, fibers may be impregnated with a liquid which, at room temperature is a non-solvent therefor, but which at a higher or lower temperature is capable of activating the potentially adhesive fibers.

Also when the mats, webs, or the like comprise thermoplastic fibers, they may be activated by subjecting them to steam, with or without pressure, especially where it is desired to produce a product characterized by extreme softness, low density, and relatively great thickness. It is also possible to activate the activatable fibers present in the fibrous web or mat by subjecting the same to a high frequency electric current as disclosed in the co-pending application of Frederick C. Wedler Serial No. 512,489, filed December 1, 1943, now abandoned.

A plasticizer may be applied to the fibers and/or to the product before partial activation. The plasticizer may function to increase the flexibility of the fibers and, when employed with thermoplastic fibers, the plasticizer may serve, in addition, to lower the thermal softening point. The plasticized thermoplastic fibers can be rendered adhesive by heating to a temperature below that at which the non-thermoplastic textile fibers associated therewith would be detrimentally affected by such heating. The plasticizer may be allowed to remain in the product, or it may be removed by suitable treatment, such as washing and extraction, thus again elevating the thermal softening point of the thermoplastic material and preventing reactivation upon ironing.

During or after partial activation, the products may be compacted, if it is desired to produce a web of increased density, and the compacting may be effected in any suitable manner, as by pressing, squeezing, and tensioning. For example, the mechanically applied pressure exerted on the activated material during and/or after activation, and/or during calendering, embossing, printing, or dyeing will effect compacting of the fibers. Also, the fibrous mat or web, in activated condition, may be passed between pressure rolls to compress the mixed fibers, or it may be subjected to tension in one or both directions.

The partially set or bonded web or bat may then be placed on one or both sides of a textile fabric and the fibers drawn partly through the fabric by means of barbed needles, after which the product is subjected to heat and pressure to further activate the inherent tackiness of the potentially adhesive fibers and cause a permanent adhesion of the fibers in the bat or bats and anchoring of the felt-like bat or bats to the fabric base. As an alternative, the commingled fibers in unfeated condition that is, without any activation of the potentially adhesive fibers may be placed on one or both sides of a textile fabric reinforcement and needled thereto in the usual manner, after which the product is subjected to heat and pressure to effect activation of the potentially adhesive fibers and binding of the fibers in the product, and of the layer or layers of bonded fibers to the fabric base.

Instead of needling the partially felted or un-felted bat to the fabric support, the bat may be plated on the surface of the fabric. In this embodiment the surface of the fabric may be provided with a layer of liquid adhesive material or with a fibrous layer which preferably comprises potentially adhesive fibers or such fibers admixed with non-adhesive fibers, which layer assists in anchoring the felt-like bat to the fabric. The pre-formed bat which may or may not have been subjected to treatment to effect a partial activation of the potentially adhesive fibers is placed on the layer or sheeting of adhesive material or fibers, and the whole subjected to heat and pressure to effect a firm binding together of the fibers in the bat and to secure a permanent adhesion and anchoring of the bat to the fabric.

According to the preferred embodiment of the invention, a layer of binding material consisting of or comprising potentially adhesive fibers is applied to at least one surface of a textile fabric, and commingled potentially adhesive fibers and non-adhesive fibers are air-deposited thereon, and the whole is subjected to heat and pressure to effect binding together of the fibers and of the various layers making up the composite product. The fabric may comprise potentially adhesive fibers, or mixtures thereof with non-adhesive fibers, all of the potentially adhesive fibers, wherever they occur in the composite structure, being simultaneously activated to thereby bind fibers together throughout the entire structure. Preferably, the binding material disposed between the felt-like bat and the textile fabric consists of potentially adhesive fibers which are formed by spraying the fiber-forming material into a setting atmosphere, and the fibers are deposited on the fabric concurrently with their formation.

If the textile fabric reinforcement comprises either potentially adhesive fibers, or a mixture containing such fibers, the layer of binding adhesive material between the fabric and felt-like bat may be dispensed with, at least at some parts of the composite product, and the felt-like mat may be deposited directly on the fabric, after which the product may be treated to activate all of the potentially adhesive fibers occurring at all parts thereof, to bind binders therein, and to effect anchoring of the layers together. The product may be activated in any suitable manner, as previously recited herein, but the preferred method of activation involves the use of hot air currents and, where the binding material between the layers comprises potentially adhesive fibers, activation may be carried to the point where such potentially adhesive fibers lose their fibrous structure, and flow to form a continuous film of binding substance.

The potentially adhesive fibers comprising the binding layer between the felt-like bat and the fabric, and the potentially adhesive fibers comprising the fabric, if any, may be the same as or different from the potentially adhesive fibers comprising the bat. The potentially adhesive fibers comprising some of the layers making up the final composite structure may be more readily activatable and rendered tacky at a lower temperature or by a lesser period of heating than the fibers comprising remaining layers, and the layers may be assembled in such manner that those comprising the more readily activatable fibers occur at one surface of the product, or at an intermediate point therein, or the activability of the fibers may increase progressively from

one surface of the product to the other, depending upon the manner in which heat is to be applied thereto. This method of assembling the various layers is especially advantageous where it is desired to simultaneously activate the potentially adhesive fibers at all parts thereof, and where it is desired to activate the fibers comprising the binding layer between adjacent textile fabric layers and felt-like layers to the extent that such fibers flow to form a continuous film, while merely softening or deforming the fibers at other parts of the product to cause the same to coalesce by interlocking together.

However the felt-like bat and fabric are anchored together, after activation, and compacting, if the latter is employed, the product is treated to deactivate the adhesive fibers, that is to render the adhesive fibers non-tacky so as to fix the new relationship of the mixed fibers throughout and at all parts of the composite product, wherever the adhesive fibers occur. If activation has been accomplished by heat, deactivation may be accomplished by cooling, or by heating at the same temperature for a prolonged period, or at a higher temperature, in the case of thermosetting resins; and if activation is by means of a solvent, deactivation may involve extraction of the solvent as by washing, evaporation, or decomposition.

In the drawing there is shown apparatus suitable for practicing the invention.

Figure 1 is a side elevation of one embodiment of suitable means for carrying out the preferred form of the invention;

Figure 2 is a side elevation of another embodiment of means for carrying out the invention;

Figure 3 is a plan view of an article in accordance with the invention;

Figure 4 is a plan view of another type of article according to the invention; and

Figure 5 is a plan view of still another article according to the invention.

When using the apparatus shown in Figure 1, a textile fabric 2, is unwound from roller 2a, and is then carried by an endless belt 3, which is made of flexible material such as textile, metal, leather, or the like, which belt is preferably positioned in a horizontal plane at the base of chamber 4. Preferably belt 3 is provided with a multiplicity of small uniformly distributed perforations and runs continuously over a similarly uniformly perforated false bottom or screen 5. As belt 3 passes under chamber 4, a composition suitable for forming potentially adhesive fibers is dispersed by means of the spray gun 6 into a gaseous atmosphere contained in chamber 4. Any material which is not formed into fibers is caught on shelf 7 and may be removed at intervals. Solvent may be removed from chamber 4 through a screened vent 8 by means of a suction device (not shown). The potentially adhesive fibers thus formed are deposited on the surface of fabric 2. The fabric is then carried by belt 3 from chamber 4 into chamber 9.

Potentially adhesive fibers are formed by spraying a suitable composition into chamber 10 by spray gun 11. Any material which is not formed into fibers is caught on shelf 12. Solvent may be removed from chamber 10 through a screened vent 13 by means of a suction device (not shown). The potentially adhesive fibers thus formed are withdrawn from chamber 10 and blown into chamber 9 through conduit 14 by blower 15. Simultaneously, a multiplicity of non-adhesive fibers are blown into chamber 9, preferably in a

direction opposite to that of the potentially adhesive fibers through conduit 16 by blower 17. The fibers are scattered about in chamber 9 by the turbulence of the air streams, and are thoroughly mixed together before settling out. The two types of fibers are thus brought together at a point sufficiently removed from the point of deposition to permit good commingling during deposition. The mixed fibers then come to rest on the layer of potentially adhesive fibers distributed on the surface of fabric 2. Air may be permitted to escape from chamber 9 through a screened exhaust pipe 18.

The product 19, comprising the various layers is carried on belt 3 from chamber 9. Positioned along the path of travel of belt 3 is an endless foraminous belt 20. The belt 3 and product 19 pass between rollers 21 and 22 and through a heating zone. As the product passes through such zone, air drawn into heating cabinet 23 through inlet 24 is directed onto product 19 by means of conduit 25 through the action of blower 26. The heated air is drawn downwardly through the product by means of the exhaust pump 27 and discharged to the atmosphere.

The product 19, in which the potentially adhesive fibers are now in activated condition, passes from the heating zone between rollers 28 and 29 and directly into a confined cooling or deactivating zone, at which point cool air is directed on the product by blower 30 through conduit 31 and drawn downwardly therethrough by means of exhaust blower 32.

The product undergoes a certain amount of compacting as it leaves chamber 9, and hence decreases in thickness as it passes through the heating zone, and the rollers 28 and 29 may be suitably adjusted to take into account such changes in the product due to the force or the air current thereon. Rolls 28 and 29 may be spaced apart so that they serve merely to assure confinement of the product 19 between the belts in the heating zone without exerting substantial pressure thereon; or they may be adjusted to apply a substantial compacting pressure to reduce the product so that the bat of interfelted fibers is of any thickness and density desired. Rolls 33 and 34 are preferably spaced apart the same distance as rolls 28 and 29 so that these two pairs of rolls cooperate to maintain the proper thickness of the product 19 during cooling. Additional pairs of rolls may be interposed between the pairs 28, 29 and 33, 34 to assure that the desired thickness is produced.

When using the apparatus shown in Figure 2, a composition for forming potentially adhesive fibers is dispersed into a setting medium contained in chamber 35 through spray gun 36. Material which does not form fibers is collected on shelf 37 and recovered at intervals; solvent is removed through screened vent 38 by means of a suction device, (not shown). Simultaneously, a multiplicity of non-adhesive fibers are blown into chamber 35 through conduit 39 by blower 40. The mixed fibers come to rest on the surface of endless belt 41 made of flexible material such as textile, metal, leather, etc., which belt is positioned in a horizontal plane at the base of chamber 35. Preferably, belt 41 is foraminous or provided with a plurality of small uniformly spaced perforations and runs over a similarly constructed screen 42. A suction pump 43 is connected to the region below the belt in chamber 35 to create a down draft through belt 41 as it passes through the chamber. As the fibers are

deposited on one portion of the belt, the suction at other points thereof is increased so that the intermingled fibers are drawn downwardly through chamber 35 onto successive portions of belt 41, which assists in a uniform distribution of the fibers over the belt surface, and results in the production of a bat or web of uniform thickness throughout.

The bat 44 is carried on the belt 41 from chamber 35, past rollers 45, 46 from which a fabric 47 consisting of potentially adhesive fibers is unwound and laid upon bat 44.

The bat 44 carrying fabric 47 is carried on belt 41 through chamber 48. A potentially adhesive fiber-forming composition is dispersed in chamber 48 by gun 49. Any material which does not form fibers is caught on shelf 50; solvent is removed through a screened vent 51 by suction means (not shown). Simultaneously, a multiplicity of non-adhesive fibers are blown into chamber 48 through conduit 52 by blower 53. The fibers which are commingled in chamber 48, finally come to rest in the form of a mixed fibrous bat on the top of fabric 47, to form a product consisting of two bats of interfelted fibers disposed on the respective surfaces of fabric 47.

The composite product is carried from chamber 48 on belt 41. Positioned along the path of the belt 41 is an endless screen belt 54. The product and belt pass between rollers 55 and 56 and through a heating zone. As it passes through such zone, air drawn into heating cabinet 57 through inlet 58 is directed to the product by means of conduit 59 through blower 60. The heated air is drawn downwardly through the product by means of the exhaust pump 61 and discharged to the atmosphere. The product, in which all of the potentially adhesive fibers occurring at all parts thereof are now in activated condition, passes from the heating zone through rollers 62 and 63 and directly into a confined cooling or deactivating zone, at which point cool air is directed on the product by blower 64 through conduit 65, and drawn downwardly therethrough by means of exhaust blower 66.

The product comprising the two bats of interfelted fibers disposed on opposite surfaces of the fabric reinforcement, undergoes a certain amount of compacting and hence decreases in thickness as it passes through the heating zone, and the rollers 62 and 63 may be suitably adjusted to take into account such changes in the bats due to the force of the air current thereon. Rolls 62 and 63 may be spaced apart so that they serve merely to assure confinement and contact of the product between the belts in the heating zone without exerting substantial pressure thereon, or they may be adjusted to apply a substantial compacting pressure to reduce the bats to any thickness desired. Rolls 67 and 68 may be spaced apart the same distance as rolls 62 and 63 so that these two pairs of rolls cooperate to maintain the proper thickness of the product during cooling.

Figure 3 illustrates a product according to the invention, which comprises a bat 69 of interfelted potentially adhesive fibers and non-adhesive fibers in which the fibers are bonded together due to the tackiness of the potentially adhesive fibers after activation, one surface of the bat being exposed, and the other surface being anchored to a textile fabric support 70 by means of an adhesive layer 70a.

Figure 4 illustrates a 3-ply product, such as that made in accordance with Figure 2, in which

bats 71 and 72 are disposed on opposing surfaces of fabric 73, and Figure 5 illustrates a multi-layer product, in which textile fabric supports 74 and 75 are disposed between bats of interfelts fibers 76, 77 and 78. In all cases, the felts webs or bats comprise bonded fibers as described hereinabove.

The ratio of potentially adhesive fiber to other fiber used in the felt-like layer and/or the fabric layer may also vary widely depending on the properties of the two types of fibers and may be regulated to suit the purpose for which the product is destined, but in general a minor proportion, preferably from 5 per cent to 45 per cent, usually from 5 per cent to twenty per cent, of the synthetic resin fiber will be employed. This minor proportion is generally sufficient even when the non-adhesive fibers are extremely short, the reinforcement or support provided by the textile fabric being especially valuable in such constructions. When a greater degree of strength or a closer bonding of the component fibers is desired, their percentage may be relatively high, whereas in soft felts in which it is desirable to have a comparatively small amount of bonding of the component fibers, the percentage will be relatively small.

The products may be used as flat felts, per se, or they may be molded or shaped over three-dimensional objects and are particularly useful for such latter purposes since they may be drawn fairly tautly over objects or surfaces having rounded or squared contours or other configuration departing from a simple single-plane flat surface while maintaining continuity of the interfelts structure and without bursting or tearing. Thus the products may be used as fillers for various purposes, as fillers for chair cushions, or other pieces of upholstery, and their ability to undergo flexing when associated with springs or the like without tearing and resultant lumpiness is particularly advantageous when the products are so used. The laminated products comprising the organic fibers may also be used as acoustic aids, for example, sound deadeners, or as heat insulators, shock absorbers, rug or carpet linings, etc. Products useful as shoe stiffeners may be obtained, and in that case the anchoring layer preferably comprises permanently thermosetting fibers, while the fibers comprising the felt-like bat and the reinforcing fabric are permanently thermoplastic.

The invention has the advantage that very light weight, thick, felt-like structures may be obtained which are characterized by low density, high porosity and permeability, without sacrifice of firmness or tensile strength. Inexpensive products may be manufactured from short fibers occurring in waste materials without requiring the utilization of an unduly large percentage of potentially adhesive fibers, and the products may be subjected to severe flexing and bending stresses and strains without disintegration or tearing at any part thereof. The invention is also of special advantage for the production of products of cloth-like character and it is possible to make use of short, waste fibers, such as wool waste, and obtain cloth-like products having substantially all the benefits of a wool fabric, such as warmth, feel, and the like.

Since changes may be made in practicing the above invention without departing from the spirit and scope thereof, it is to be understood that the foregoing description and specific illustrations are given by way of exemplification only, and the in-

vention is not to be limited except as defined by the appended claims.

I claim:

1. In a process for producing a composite product having the external appearance and characteristics of a felt-like product and comprising at least one layer of textile fabric comprising interlaced yarns and at least two layers of felt-like material, in which one surface of two of the felt-like layers is exposed and the other surface thereof is substantially permanently anchored to a layer of the textile fabric, the steps comprising depositing a multiplicity of discontinuous potentially adhesive fibers on both faces of the textile fabric, superimposing thereon a mixture of non-adhesive fibers and potentially adhesive fibers, and activating the potentially adhesive fibers to effect a binding together of the non-adhesive fibers by the activated potentially adhesive fibers wherever the latter occur in the composite product.
2. In a process for producing a composite product having the external appearance and characteristics of a felt-like product and comprising at least one layer of textile fabric comprising interlaced yarns and at least two layers of felt-like material, in which one surface of two of the felt-like layers is exposed and the other surface thereof is substantially permanently anchored to a layer of the textile fabric, the steps comprising depositing a multiplicity of discontinuous potentially adhesive fibers on both faces of the textile fabric, superimposing thereon a mixture of non-adhesive fibers and potentially adhesive fibers, and activating the potentially adhesive fibers to effect a binding together of the non-adhesive fibers by the activated potentially adhesive fibers wherever the latter occur in the composite product.
3. In a process for producing a composite product having the external appearance and characteristics of a felt-like product and comprising at least one layer of textile fabric comprising interlaced yarns and at least two layers of felt-like material, in which one surface of two of the felt-like layers is exposed and the other surface thereof is substantially permanently anchored to a layer of the textile fabric, the steps comprising depositing a multiplicity of discontinuous potentially adhesive fibers on both faces of the textile fabric, superimposing thereon a mixture of non-adhesive fibers and potentially adhesive fibers, and activating the potentially adhesive fibers to effect a binding together of the non-adhesive fibers by the activated potentially adhesive fibers wherever the latter occur in the composite product and deactivating the activated fibers.
4. The process of claim 3, wherein the mixture of potentially adhesive fibers and non-adhesive fibers is air-deposited on the surfaces of the fabric carrying the potentially adhesive fibers.
5. In a process for producing a composite product having the external appearance and characteristics of a felt-like product and comprising at least one layer of textile fabric comprising interlaced yarns and at least two layers of felt-like material, in which one surface of two of the felt-like layers is exposed and the other surface thereof is substantially permanently anchored to a layer of the textile fabric, the steps comprising forming a potentially adhesive, fiber-forming plastic material into a multiplicity of discontinuous fibers, depositing such fibers concurrently with their formation on both surfaces of a textile fabric; commingling a multiplicity of discontinuous potentially adhesive fibers with a multiplicity of non-adhesive fibers, depositing the mixed fibers on the fabric surfaces carrying the first-mentioned potentially adhesive fibers, and activating the potentially adhesive fibers to effect a binding together of the non-adhesive fibers by the activated potentially adhesive fibers wherever the latter occur in the composite product.
6. In a process for producing a composite product having the external appearance and characteristics of a felt-like product and comprising at least one layer of textile fabric comprising interlaced yarns and at least two layers of felt-like material, in which one surface of two of the felt-like layers is exposed and the other surface thereof is substantially permanently anchored to a layer of the textile fabric, the steps comprising forming a potentially adhesive, fiber-forming

plastic material into a multiplicity of discontinuous fibers, depositing such fibers concurrently with their formation on both surfaces of a textile fabric comprising potentially adhesive fibers, commingling a multiplicity of discontinuous potentially adhesive fibers with a multiplicity of non-adhesive fibers, depositing the mixed fibers on the fabric surfaces carrying the first-mentioned potentially adhesive fibers, and activating the potentially adhesive fibers to effect a binding together of the non-adhesive fibers by the activated potentially adhesive fibers wherever the latter occur in the composite product.

6. The process of claim 5, wherein the mixture of potentially adhesive and non-adhesive fibers is air-deposited on the surfaces of the fabric carrying the potentially adhesive fibers.

7. In a process for producing a composite product having the external appearance and characteristics of a felt-like product and comprising at least one layer of textile fabric comprising interlaced yarns and at least two layers of felt-like material in which one surface of two of the felt-like layers is exposed and the other surface thereof is substantially permanently anchored to a layer of the textile fabric, the steps comprising forming a potentially adhesive, fiber-forming plastic material into a multiplicity of discontinuous fibers, depositing such fibers concurrently with their formation on both surfaces of a textile fabric; separately forming a potentially adhesive fiber-forming plastic material into a multiplicity of discontinuous fibers, associating the last-mentioned potentially adhesive fibers concurrently with their formation with a multiplicity of discontinuous non-adhesive fibers, depositing the mixed fibers on the fabric surfaces carrying the first-mentioned potentially adhesive fibers, and activating the potentially adhesive fibers to effect a binding together of the non-adhesive fibers by the activated potentially adhesive fibers wherever the latter occur in the composite product.

8. In a process for producing a composite product having the external appearance and characteristics of a felt-like product and comprising at least one layer of textile fabric comprising interlaced yarns and at least two layers of felt-like material in which one surface of two of the felt-like layers is exposed and the other surface thereof is substantially permanently anchored to a layer of the textile fabric, the steps comprising forming a potentially adhesive, fiber-forming plastic material into a multiplicity of discontinuous fibers, depositing such fibers concurrently with their formation on both surfaces of a textile fabric comprising potentially adhesive fibers, separately forming a potentially adhesive fiber-forming plastic material into a multiplicity of discontinuous fibers, associating the last-mentioned potentially adhesive fibers concurrently with their formation with a multiplicity of discontinuous non-adhesive fibers, depositing the mixed fibers on the fabric surfaces carrying the first-mentioned potentially adhesive fibers, and activating the potentially adhesive fibers to effect a binding together of the non-adhesive fibers by the activated potentially adhesive fibers wherever the latter occur in the composite product.

9. A composite, reinforced, felt-like product comprising at least one layer of textile fabric comprising interlaced yarns and at least two layers of felt-like material each formed from a mixture of short leather fibers and discontinuous potentially adhesive fibers which occur at substan-

tially all portions of the felt-like layers, the fibers in the felt-like layers being autogenously bonded together, said layers being assembled so that one surface of two of the felt-like layers is exposed and all of the layers being substantially permanently anchored together solely by adhesion at their surfaces.

10. A composite, reinforced, felt-like product comprising at least one layer of textile fabric comprising interlaced yarns and at least two layers of felt-like material each formed from a mixture of cotton linters and discontinuous potentially adhesive fibers, the fibers in the felt-like layers being autogenously bonded together, said layers being assembled so that one surface of two of the felt-like layers is exposed and all of the layers being substantially permanently anchored together solely by adhesion at their surfaces.

11. A composite, reinforced, felt-like product comprising at least one layer of textile fabric comprising interlaced yarns and at least two layers of felt-like material each formed from a mixture of shear flock and discontinuous potentially adhesive fibers, the fibers in the felt-like layers being autogenously bonded together, said layers being assembled so that one surface of two of the felt-like layers is exposed and all of the layers being substantially permanently anchored together solely by adhesion at their surfaces.

12. A composite, reinforced, felt-like product comprising at least one layer of textile fabric comprising interlaced yarns, at least two layers of felt-like material each formed from a mixture of short leather fibers and discontinuous potentially adhesive fibers, the fibers in the felt-like layers being autogenously bonded together, and a layer of adhesive material disposed between each layer of fabric and each layer of felt-like material, said layers being assembled so that one surface of two of the felt-like layers is exposed and all of the layers being substantially permanently anchored together solely by adhesion at their surfaces.

13. A composite, reinforced, felt-like product comprising at least one layer of textile fabric comprising interlaced yarns, at least two layers of felt-like material each formed from a mixture of cotton linters and discontinuous potentially adhesive fibers, the fibers in the felt-like layers being autogenously bonded together, and a layer of adhesive material disposed between each layer of fabric and each layer of felt-like material, said layers being assembled so that one surface of two of the felt-like layers is exposed and all of the layers being substantially permanently anchored together solely by adhesion at their surfaces.

14. A composite product having the external appearance and characteristics of a felt-like product and comprising at least one layer of textile fabric comprising interlaced yarns, at least two layers of felt-like material formed from a mixture of shear flock and potentially adhesive fibers, the fibers in the felt-like layers being autogenously bonded together, and a layer of adhesive material disposed between each layer of fabric and each layer of felt-like material, said layers being assembled so that one surface of two of the felt-like layers is exposed and the other surface thereof is substantially permanently anchored to one surface of a layer of the textile fabric.

15. A composite, reinforced, felt-like product comprising at least one layer of a textile fabric comprising interlaced yarns and at least one layer of felt-like material, disposed on each surface of

15

the fabric, each of the felt-like layers being formed from a mixture of discontinuous, non-adhesive fibers and discontinuous, potentially adhesive fibers which occur at substantially all portions of the felt-like layers and have an inherent tackiness on heating, the fibers in the felt-like layers being autogenously bonded together, and all of the layers of the product being substantially permanently anchored together solely by adhesion at their surfaces.

16. A product as in claim 15 wherein the fabric comprises potentially adhesive fibers.

17. A composite, reinforced, felt-like product comprising at least one layer of textile fabric comprising interlaced yarns, at least one layer of felt-like material disposed on each surface of the fabric, and a layer of adhesive material disposed between the layer of fabric and each felt-like layer, each of the felt-like layers being formed from a mixture of discontinuous non-adhesive fibers and discontinuous potentially adhesive fibers which occur at substantially all portions of the felt-like layers and have an inherent tackiness on heating, the fibers in the felt-like layers being autogenously bonded together, and all of the layers of the product being substantially permanently anchored together solely by adhesion at their surfaces.

18. A product according to claim 17, wherein the layer of adhesive material disposed between the fabric layer and each felt-like layer comprises potentially adhesive fibers.

19. A process for producing a composite, reinforced, product having the external appearance and characteristics of a felt-like product and comprising at least one layer of textile fabric

16

comprising interlaced yarns and at least one layer of felt-like material disposed on each surface of the fabric, each of the felt-like layers comprising a mixture of discontinuous potentially adhesive fibers having an inherent tackiness on heating and discontinuous non-adhesive fibers, and in which the fibers in the felt-like layers are autogenously bonded together, the step which comprises intimately associating the potentially adhesive and non-adhesive fibers, assembling the mixture of fibers and at least one fabric into a structure the exposed surfaces of which comprise the mixed fibers in felt-like form, and activating the potentially adhesive fibers to effect a bonding together of the non-adhesive fibers by the potentially adhesive fibers wherever they occur in the product and produce a product in which the layers are substantially permanently anchored together solely by adhesion at their surfaces.

CARLETON S. FRANCIS, JR.

## REFERENCES CITED

The following references are of record in the file of this patent:

## UNITED STATES PATENTS

| Number    | Name          | Date          |
|-----------|---------------|---------------|
| 171,728   | Howard        | Jan. 4, 1876  |
| 292,187   | Tyler         | Jan. 22, 1884 |
| 906,044   | Malcolm       | Dec. 8, 1908  |
| 921,674   | Clark         | May 18, 1909  |
| 2,202,025 | Reed          | May 28, 1940  |
| 2,331,321 | Heaton        | Oct. 12, 1943 |
| 2,336,745 | Manning       | Dec. 14, 1943 |
| 2,385,870 | Lashar et al. | Oct. 2, 1945  |